

# UNITED STATES PATENT OFFICE.

STERLING ELLIOTT, OF NEWTON, MASSACHUSETTS.

## PROCESS OF MAKING ALLOYS OF ZINC WITH COPPER.

No. 927,843.

Specification of Letters Patent.

Patented July 13, 1909.

Application filed October 12, 1908. Serial No. 457,284.

*To all whom it may concern:*

Be it known that I, STERLING ELLIOTT, of Newton, county of Middlesex, State of Massachusetts, have invented an Improvement in Processes for Making Alloys of Zinc with Copper, of which the following is a specification.

This invention relates to an improved process for producing an alloy of zinc with copper.

The object of the invention is the production of the alloy at a temperature much less than the melting point of copper, whereby the expense of production is very materially decreased and numerous other advantages gained incident to the employment of the greatly reduced temperature as compared with the temperature ordinarily employed.

In carrying out my process I first melt the zinc, then add the copper to the molten zinc and then raise the temperature to the melting point of the alloy which is to be produced or thereabout which is less than the melting point of copper and also less than the boiling point of zinc. The affinity of the zinc for the copper causes the latter to be absorbed or dissolved to some extent even when the zinc is barely melted, and this effect is more marked in proportion as the

pieces of copper are smaller in size, for the reason that a greater surface of copper will be exposed to the action of the molten zinc. However, I continue to raise the temperature of the mass until it reaches the melting point of the alloy which is to be produced or thereabout, to obtain an alloy having a perfectly homogeneous structure. For exam-

ple; assuming the melting point of zinc to be 412° C. and its boiling point 1040° C. and the melting point of copper to be 1090° C. 40 and the melting point of the alloy which is to be produced to be 973° C. it will be noted that when the copper is placed in the molten zinc at 412° C. it begins to dissolve, but even so the temperature is raised to 973° C. or 45 thereabout, which, it will be noted is less than the melting point of the copper and also less than the boiling point of the zinc, yet is high enough to produce an alloy having a perfectly homogeneous structure. In 50 carrying out my process the zinc and subsequently the alloy will be covered with any well-known or suitable flux, such, for instance as charcoal or borax.

Having thus described my invention, what 55 I claim as new and desire to secure by Letters Patent is:—

The process herein described of producing an alloy of zinc with copper, which consists in first melting the zinc, then adding the copper to the molten zinc and raising the temperature to the melting point of the alloy which is to be produced or thereabout, which is less than the melting point of the copper and also less than the boiling point 60 of the zinc. 65

In testimony whereof, I have signed my name to this specification, in the presence of two subscribing witnesses.

STERLING ELLIOTT.

Witnesses:

B. J. NOYES,  
H. B. DAVIS.